

# UNITED STATES PATENT OFFICE.

JOHN M. TIPPETT, OF COLORADO SPRINGS, COLORADO.

## PROCESS OF EXTRACTING PRECIOUS METALS AND OTHER METALS FROM ORE.

1,236,501.

Specification of Letters Patent. Patented Aug. 14, 1917.

No Drawing.

Application filed December 23, 1916. Serial No. 138,631.

*To all whom it may concern:*

Be it known that I, JOHN M. TIPPETT, a citizen of the United States, and a resident of Colorado Springs, in the county of El Paso and State of Colorado, have invented 5 certain new and useful Improvements in Processes of Extracting Precious Metals and other Metals from Ore, of which the following is a specification.

10 This invention relates to a process for the treatment of the ores of the precious metals (gold and silver) and has for its object the extraction of as large a proportion as possible of the precious metals contained in the 15 ore and at the same time recovering any base metals, such as copper, lead, zinc, iron, etc., which may be present in the ore.

I have discovered that by following the 20 procedure hereinafter detailed, it is possible to accomplish oil flotation in a cyanid solution. By combining oil flotation with the steps of the cyanid process, I have produced a process of extracting which is more 25 efficient and also more economical than previous methods of treating the ores of precious metals. The process is applicable to any gold or silver ores, and is particularly adapted to the treatment of ores from the Cripple Creek district in Teller county, 30 Colorado.

In order that my invention may clearly be understood, I shall proceed to describe in detail a specific embodiment of it, as well as some modifications of the embodiment 35 first described. It should be clearly understood, however, that my invention is by no means limited to the particular embodiments described in detail.

The ore to be treated is first broken or 40 crushed to a suitable size for fine grinding. The ore is then mixed with a solution of cyanid of potassium or sodium (KCN or NaCN). Equal quantities of ore and solution are used. The strength of the solution 45 varies according to the nature of the ore to be treated from one-quarter of a pound to four pounds of the cyanid salt to one ton of water. The ore and cyanid solution are then fed to a tube mill, a ball mill, a Chilian 50 mill, or stamp, where the ore is finely comminuted.

While the ore and the cyanid solution are 55 passing into the mill an alkali or a mixture of alkalis is added to the ore. The amount of alkali depends upon the acidity of the ore under treatment. It will vary from one-half

pound to ten pounds per ton of ore. It is not necessary that any particular alkali be used, although I have found caustic soda (NaOH) preferable. Sodium carbonate 60 (Na<sub>2</sub>CO<sub>3</sub>), or lime (CaO), or a mixture of the three alkalis mentioned, or any two of them, is satisfactory. The adding of the alkali or alkalis serves two purposes: It prevents the cyanid from being consumed 65 should the pulp become too acid on account of the acidity of the ore, and I have found it is of material assistance in effecting flotation.

As the ore and cyanid solution enter into 70 the mill, I add a suitable flotation oil, the amount of which may vary from one-half pound to four pounds per ton of ore.

The ore, the cyanid solution, the alkalis and the oil are mixed together in the grinding mill. The oil emulsifies during the grinding and coats the sulfids and metallic particles present. After the grinding has reduced the ore to the degree of fineness usual for cyanid treatment, the mixture is 80 drawn from the mill and additional cyanid solution of the same strength previously used is added, making the ratio of ore to solution one to three or one to four. The mixture is then flowed to a flotation cell, such 85 as the Callow pneumatic cell or the minerals separation cell, where a large portion of the richest and finest minerals, including both sulfids and metallic particles, are floated by the gas bubbles produced in the mixture in 90 the flotation cell and removed from the pulp as a concentrate. The minerals recovered by this flotation step are those which are so fine that table concentration cannot save them. These concentrates are very difficult 95 to treat in the cyanid solution if not removed.

The tailings from the flotation cell are passed over gravity concentration tables, which may be of the well known Wilfley 100 type. There the coarser particles of mineral which flotation failed to recover are separated from the pulp.

The tailings from the concentration tables pass into thickening tanks of the Dorr 105 type. The clear solution overflowing from the thickening tanks is treated with zinc to precipitate the gold and silver in the usual manner. The underflow from the thickeners, containing the pulp, flows to agitating 110 tanks of the sort usually used in connection with the cyanid process. After agitation,

the pulp may be passed through any recognized type of slime filter to remove the gold and silver solution from the ore. The solution is then treated with zinc to precipitate the gold and silver contained in it.

Changes may be made in the details of the process described without departing from my invention. For example, it is not necessary that the flotation oil be added to the ore before the ore enters the grinding mill. It may be added after the ore has been finely ground and emulsified by agitation, either in a mechanical oil flotation cell, or an agitation tank before reaching the flotation cell.

I claim as my invention:—

1. An improvement in the cyanid process for treating ores, comprising the step of separating out a portion of the values in the ore by flotation in the presence of the cyanid solution.

2. An improvement in the cyanid process for the treatment of ores, comprising mixing the ore with cyanid solution and oil, and separating a portion of the values from the mixture by flotation.

3. An improvement in the cyanid process for the treatment of ores, comprising mixing the ore with cyanid solution and oil and alkali; emulsifying the oil in the presence of the ore, the alkali, and the cyanid solution; floating a portion of the values in the pulp by producing gas bubbles in the mixture, and removing the values floated.

4. An improvement in the cyanid process of treating ores, comprising mixing the ore with an equal or greater amount of cyanid solution, alkali sufficient in quantity to

counteract the acidity of the ore, and a quantity of oil amounting to a fraction of one per cent. of the ore; emulsifying the oil in the presence of the ore, the alkali and the cyanid solution; and producing gas bubbles in the mixture whereby a portion of the values are floated.

5. An improvement in the cyanid process of treating ores, comprising mixing the ore with cyanid solution and oil, and flowing the resulting mixture to a grinding mill, and then to a flotation cell.

6. An improvement in the cyanid process of treating ores, comprising mixing cyanid solution, oil, and alkali with the ore; and passing the resulting mixture to a grinding mill, and then to a flotation cell.

7. An improvement in the cyanid process of treating ores, comprising mixing the ore with an equal quantity of cyanid solution, alkali sufficient to counteract the acidity of the ore, and an amount of oil equal to a fraction of one per cent. of the ore; passing the resulting mixture through a grinding mill; adding additional cyanid solution; and passing the mixture to a flotation cell.

8. A process for the treatment of ores, comprising mixing the ore with cyanid solution and oil, emulsifying the oil, passing the mixture through a flotation cell where a portion of the minerals are separated out and removed, passing the remaining mixture over concentrating tables where a further portion of the minerals are separated out, separating the solids remaining in the mixture from the solution, and precipitating the values dissolved in the solution.

JOHN M. TIPPETT.